

Jan. 10, 1933.

L. L. GILBERT

1,893,669

SHEET FOR SANITARY AND SURGICAL PURPOSES AND METHOD OF MAKING THE SAME

Filed June 19, 1929

FIG. 1



FIG. 2



FIG. 3

Levi L. Gilbert.

Charlesville

Mass.

U.S. Pat. Off.

## UNITED STATES PATENT OFFICE

LEVI L. GILBERT, OF MUSKEGON, MICHIGAN

## SHEET FOR SANITARY AND SURGICAL PURPOSES AND METHOD OF MAKING THE SAME

Application filed June 19, 1929. Serial No. 372,109.

This invention relates to a sheet for sanitary and surgical purposes and a method of making the same which sheet is formed from paper as a composite sheet one of which 5 sheets at least is preferably of white paper.

Attempts have been made to make surgical sheets of paper which are sanitary and waterproof in order that such sheets may be sold at low prices and discarded after first use.

10 There have been no successful composite sanitary sheets of paper made for the reason that no adequate means for waterproofing and sterilization have been discovered whereby a composite sheet may be made with at least one of the sheets of white paper. Doctors prefer a white surface in sanitary sheets.

This invention is directed to a sheet made of paper in composite form with at least one of the sheets preferably of white paper to

20 together with a method of making the same and is directed to a composite sheet wherein two sheets of paper one of which is preferably of white paper are rolled together with asphalt between the two sheets in the presence of heat

25 of such a temperature as will not only melt the asphalt but will sterilize the paper. The preferred temperature being approximately 450° F.

An object of this invention is to provide a 30 method of making a composite sheet of paper for surgical purposes which is sanitary and waterproof.

Another object of the invention is to provide a composite sheet made of paper, waterproofed and sterilized which may be used for 35 surgical and sanitary purposes.

A further object of the invention is to provide a sanitary sheet for surgical purposes and the like which is economical to manufacture and which is discarded after a single 40 use.

A yet further object of the invention is to provide a composite sanitary sterilized sheet with at least one side of white paper.

45 Another and still further object of the invention is to provide a composite sheet of two single sheets of paper one of which is preferably of white paper rolled together with asphalt, or other waterproofing material, between the two single sheets under pres-

sure and in the presence of a sterilizing temperature.

The above, other, and further objects of the invention will be apparent from the following description accompanying drawing, 55 and appended claim.

According to the invention a composite sheet is formed by the method of rolling together two single sheets of paper one of which is preferably of white paper with 60 asphalt or other suitable waterproofing material or binder between the same in the presence of such heat as will not only melt the asphalt or other binder as to make the same highly fluid for adhesive purposes but at 65 the same time thoroughly sterilizes the paper so that articles may be made from the same for sanitary and surgical purposes.

The accompanying drawing illustrates an 70 embodiment of the invention and diagrammatically represents a composite sheet made in accordance with this invention, the drawing being greatly exaggerated for the purpose of clearness.

Figure 1 is an enlarged fragmental sectional view thru a composite sheet constructed in accordance with this invention. 75

Figure 2 is a perspective view of a pan 80 constructed of composite paper of this invention.

The method of this invention contemplates the provision of two suitable sheets of paper at least one of which is preferably of white paper and rolling these two sheets together with asphalt between the same for adhesive 85 purposes and, in the rolling, subjecting the same to a high heat of approximately 450° F. which not only liquefies the asphalt to such an extent as to make complete union of the two sheets of paper but at the same time thoroughly and completely sterilizes the paper. 90

Articles such as bed pans, kelleys, sanitary sheets, aprons and the like may be made from composite paper made in accordance with 95 this invention and discarded after a first use.

The use of the asphalt or other binder waterproofs the composite sheet so as to make it serve as a substitute for rubber sheeting in surgical and sanitary cases. 100

The sheet made in accordance with the method of this invention includes two portions 1 and 2 of thin paper one of which preferably the portion 1 is of white paper.

5 These two sheets are rolled together with a very thin layer of asphalt 3 between the same. The rolling is done in the presence of high heat such as 450° F. which heat completely liquefies the asphalt so as to make a 10 firm binder between the sheets 1 and 2 and at the same time thoroughly sterilizes the sheets.

15 The sheet is used with the white portion 1 uppermost and because of the use of the asphalt and the method of construction is completely waterproof.

20 Suitable articles may be made by turning back the marginal portions of a sheet to form a pan such as that illustrated in Figure 2 wherein the body of the sheet is of white paper 1 and the outer portion 2 of white paper or other paper as desired. Turning back the 25 margins as at 4 as illustrated in Figure 2 provides a dam about the margins of the sheet to prevent the escape of water or other liquids when the sheet is in use.

30 Doctor prefer and desire white paper for several reasons. First of all, the appearance of white is more pleasing than any other and furthermore, white better reflects light to aid the doctor in using the sheet of the 35 present invention. Furthermore, the white sheet shows up excretions and secretions very readily so that these can be much better examined.

40 The use of the waterproof adhesive between the two sheets of paper from which the composite article of the present invention is made and the manner of pressing together these sheets with the adhesive in between is such that the adhesive impregnates the two sheets of paper leaving the outer surfaces of the completed sheet free from shiny appearance and slippery finish so that the 45 liquids such as secretions and excretions do not run off but remain on the sheet.

50 A sheet such as that herein described is very useful for doctors as doctors may carry a supply of these composite paper sheets when making isolated calls and when through with treatment may discard the sheet without having to resterilize it as is necessary when rubber sheeting is used.

55 Oftentimes doctors are called on emergency cases requiring surgical treatment of some character necessitating the use of sanitary sheeting to protect the patient and also the table or bed on which the patient is lying.

60 Rubber sheetings, of course, are heavy and cumbersome and require sterilization and complete cleansing after every use. It is sometimes difficult for doctors or others tending emergency calls to carry a sufficient quantity of rubber sheetings for all purposes.

65 It is possible for a doctor to provide him-

self with a quantity of paper sheets made in accordance with this invention as the same occupy but very little space and when used the same may be discarded.

The use of a new sheet every time assures 70 complete sanitation without any danger whatsoever from infection from improperly disinfected or improperly sterilized rubber sheets.

The term "sterilizer temperature" as used 75 herein contemplates any temperature that destroys germs and spores and includes temperatures as high as from 385° F. to 450° F.

The composite sheet of this invention may be formed by pressing or forcing together the 80 two separate sheets in a manner other than by rolling and the claim is to be construed accordingly.

A composite sheet made in accordance with 85 this invention is flexible and pliable and smooth and has been proved to be completely waterproof or liquid-proof in use.

The invention has been described herein more or less precisely, yet it is to be understood that changes may be made in the arrangement and proportion of parts and that equivalents may be substituted without departing from the spirit and scope of the invention.

90 The invention is claimed as follows:

95 The method of making a sterilized composite paper sheet for sanitary and surgical purposes, which method comprises the placing of a thin layer of asphalt between a pair of paper sheets, then forcing said sheets and asphalt together in intimate relation in the presence of a temperature high enough to melt the asphalt and sustained to produce sterilization of the composite sheet.

100 In testimony whereof I have hereunto subscribed my name at Chicago, Cook County, Illinois.

105 LEVI L. GILBERT.

110

115

120

125

130